

Nov. 3, 1931.

D. S. GUSTIN

1,830,165

COATED LAMP BULB

Filed Dec. 10, 1927



INVENTOR  
D. S. GUSTIN

BY *M. J. Rego*  
ATTORNEY

## UNITED STATES PATENT OFFICE

DANIEL S. GUSTIN, OF BLOOMFIELD, NEW JERSEY, ASSIGNOR TO WESTINGHOUSE LAMP COMPANY, A CORPORATION OF PENNSYLVANIA

## COATED LAMP BULB

Application filed December 10, 1927. Serial No. 238,244.

This invention relates to the process of coating or to the application of a paint or the like to an incandescent lamp bulb and relates more particularly to the coating of a bulb on the interior wall thereof such as disclosed in copending application of Aaron M. Hageman and Albert F. Lindstrom, Serial No. 238,734 filed December 9, 1927 for method and apparatus for coating the interior wall of hollow bodies and assigned to the same assignee as is the present invention.

As set forth in the above mentioned pending application, lamps are sprayed with a finely divided material, preferably a composition including a pigment, a filler and a sodium silicate binder. This preparation when sprayed upon the inner wall of the bulb produces a light diffusing medium which in addition to the glossy outer surface of the bulb results in a pearly or opalescent effect.

The present invention aims to improve the light diffusing characteristics of a lamp coating as above mentioned and provides for the additional application of a film or layer of transparent or translucent substance which will improve the light transmitting properties of the layer.

The present method consists in spraying the inner surface of a bulb or other translucent hollow body with a pigment mixed with a small quantity of sodium silicate as a binder. The coated article is then subjected to a baking treatment so as to dehydrate the coating and set the same. After this initial coating has been properly set, it is again sprayed with a light diffusing coating such as kaolin to which has been added a relatively large amount of sodium silicate as a binder. This double coating of the lamp gives the same a pleasing appearance and eliminates any glare that may result as when a high temperature concentrated filamentary light source is employed.

It has been found that when coating the interior wall of a lamp bulb with a composition including sodium silicate that the sodium silicate acts to set up strains upon the surface of the bulb to such a degree that if any appreciable amount of sodium silicate is employed the bulb becomes brittle and

cracks upon a relatively small degree of impact as may be caused by handling or general transportation. It is, therefore, necessary in the initial coating of the bulb to employ a composition in which the sodium silicate is of relatively low specific gravity and good results have been obtained in which the sodium silicate binder of the initial coating has a specific gravity of about 1.025. A second or subsequent coating which has been found to give satisfactory results includes a sodium silicate binder having a specific gravity of about 1.05. This makes it possible to produce an inside coated lamp having such an amount of sodium silicate as to give the desired light diffusion to the same degree as is possible with bulbs having the coating upon the outer surface thereof in which the sodium silicate content is relatively large, inasmuch as the use of sodium silicate on the outside of the bulb has a tendency to strengthen rather than weaken the bulb.

It has further been found that upon coating lamp bulbs upon the inside surface thereof, certain of such lamps when in use tend to blacken, as for example, a lamp coating containing sienna and sodium silicate. This blackening may be due to the use of phosphorous which is employed as a getter in the lamp during the exhausting operation, the phosphorous reacting with the coating and reducing it, thus causing a blackening of the bulb.

Tests have been made using a light diffusing coating containing sodium silicate which is baked on the bulb, the coating composition containing, for example, sienna as a pigment mixed with silicate. After this coating has been baked, it was given a layer of sodium silicate. Other lamps were sprayed with sienna, kaolin and sodium silicate and also given an additional layer of sodium silicate.

It was found that when given the subsequent sodium silicate layer the lamps did not blacken or become gassy and it seems that by coating the first sprayed layer with sodium silicate the said layer is prevented from reacting with the getter as, for example, in the case of sienna and kaolin, forming a more

stable compound which does not evolve moisture. The general effect of the addition of sodium silicate to the interior of the bulb is to promote the vacuum and improve the quality of the lamp. This being true whether the sodium silicate is deposited on the coating or on other portions of the internal structure of the bulb as, for example, a deposit of sodium silicate on the stem will give 10 advantageous results.

An example of a coating composition which may be used as an initial coating may contain a filler, coloring pigment and other materials as to provide a translucent surface 15 when applied to a bulb. The coating may be prepared by mixing 250 grams of finely divided kaolin with 1000 cc. of a solution of sodium silicate having a specific gravity of about 1.025; or a coating may be prepared 20 by mixing 125 grams of kaolin with 700 cc. of a solution of sodium silicate having a specific gravity of about 1.025. The kaolin may be substituted for a color pigment or the pigment may be added to the mixture 25 which includes kaolin. It is to be understood that such quantity of pigment may be used as to give the proper depth of color to the composition. The mixture may then be placed in a ball mill mixer and milled for a 30 suitable period as, for example, about 15 hours. The coating material may be applied by pouring into a bulb or preferably by spraying as shown and described in the above mentioned copending application.

35 The bulb or the like, after the application of the coating preparation, is subjected to a relatively high degree of heat for a predetermined period of time in order that the preparation may become properly fixed to the bulb 40 surface. It has been found that by placing the bulb in an oven heated to about 150° C. and allowing it to remain there for about 2 minutes the preparation becomes firmly fixed in a satisfactory manner. After the bulb 45 has been heated and the coating has set, a second layer of sodium silicate of about 1.05 specific gravity may be applied to the initial coating. This latter layer is preferably applied while the bulb is still heated, although 50 the same may be deposited upon the initial coat after the same has cooled.

It will be understood that the exact proportions of the ingredients depends upon the light diffusing requirements of the coating and upon the color and density desired, it being understood that the foregoing example is given as one practical embodiment of the invention.

55 A bulb coated in accordance with the present invention is shown in the single figure of the accompanying drawing. As illustrated a bulb 2 may be provided with a layer 3 of light diffusing material, which layer may be encased in another layer 4 of sodium silicate as above set forth. It is obvious that al-

though the coating as shown is applied to the interior surface of the bulb, it may be applied to either the inner or the outer surface.

Although the use of a supplemental layer of sodium silicate is advantageous in enhancing the appearance of the initial coating of the bulb, it will be evident that it serves a double function in that it acts as a clean-up agent.

After a lamp bulb has been coated, it is necessary to seal the same to a lamp mount which supports the internal structure of the bulb. After the mount has been sealed into the bulb, the exhaust tube of the bulb is applied to an exhaust machine. The exhausting method includes the heating of the bulb and as an explanation of the action of the sodium silicate, it may be stated that the silicate is dehydrated when the bulb is heated up during exhaust and that when it cools down it has a high affinity for moisture. This function of the sodium silicate is important since it will reduce the tendency toward loss of vacuum in lamps, also brittle filaments and black lamps or gassy lamps.

It has been found that good results are obtained when the internal structure of the device includes an element containing a sodium silicate as, for example, a lamp having a zirconium button which contains sodium silicate as a binder, has been found to have a getter effect to hold or improve the vacuum within a sealed envelope. The dual function of the sodium silicate within an electrical device such, for example, as an internally coated incandescent electric lamp is to enhance the appearance of the coating and to permit the operativeness of the device.

As above set forth, the coating material may be what is termed a wet coating and applied by flushing or spraying. It is to be understood, however, that a so-called dry initial coating may be used; that is, the initial coating material may be in powdered form and dusted onto the interior surface of the bulb after which the sodium silicate layer may be applied. Dry coatings do not employ any binder such as sodium silicate so that when given an additional coating of sodium silicate in accordance with the present invention, a more lustrous appearance is given to the bulb. It has been the practice when dry coating bulbs to first etch the interior surface thereof and it has been found that a bulb etched and dry coated with an additional layer of sodium silicate gives a pleasing result.

Although a preferred embodiment of the invention is shown and described herein, it is to be understood that modifications may be made therein without departing from the spirit and scope of the invention as set forth in the appended claims.

What is claimed is:

1. A lamp bulb having a light diffusing

coating on a surface thereof and a layer of sodium silicate enclosing said coating.

2. A lamp bulb comprising a light diffusing coating including a filler, a sodium silicate and a sodium silicate layer enclosing said coating.

In testimony whereof, I have hereunto subscribed my name this 8th day of December 1927.

DANIEL S. GUSTIN.

5

0

5

0

15

50

55

60

65